

## UNITED STATES PATENT OFFICE

2,233,185

## ANTIFREEZE COMPOSITION

David F. Smith, Snyder, N. Y.

No Drawing. Application January 21, 1938,  
Serial No. 186,188

15 Claims. (Cl. 252—76)

This invention relates to improvements in antifreeze liquids of the type employed, for example, as heat transfer media with circulating systems.

5 One of the objects of this invention is to provide a liquid of this kind capable of efficient use at very low temperatures, which is substantially non-corrosive of metals with which the solution may contact when in use. Another object of this 10 invention is to provide a liquid of this kind comprising a solution of a readily soluble salt, which solution remains a free flowing liquid at very low temperatures, and which is substantially non- 15 corrosive of metals of the kind commonly employed in connection with circulating systems for cooling or heating liquids.

It is also an object of this invention to provide a liquid of this kind including mainly an aqueous 20 solution of an alkali metal salt of a fatty acid containing not more than nine carbon atoms per molecule. Still another object is to provide a liquid of this kind comprising mainly a solution 25 of an alkali metal salt of a fatty acid having not more than nine carbon atoms per molecule, in sufficient proportion to materially lower the freezing point of the liquid below that of water and with which certain corrosion inhibitors may 30 be mixed. It is also an object of this invention to provide a liquid comprising in the main a solution of an alkali metal salt of a fatty acid of this type, and with which may be used certain substances for reducing the wetting power or 35 creeping tendency of the liquid in contact with metal and other solid surfaces. Another object is to provide an antifreeze liquid including a salt solution of this kind in which an oil is miscible without requiring the usual emulsifying or wetting agent.

Another object of this invention is to provide 40 a method of effecting heat transfer in a cooling system, which includes the circulation of a solution of an alkali metal salt of a fatty acid having not more than nine carbon atoms per molecule and having a solidifying point far below that of 45 water and which is substantially non-corrosive of metals with which the solution contacts in a circulating system.

Other objects are to provide a method of this 50 kind including the step of circulating a slightly alkaline salt solution of this kind containing an inhibitor of corrosion; also to circulate a slightly alkaline salt solution of this kind containing a material for decreasing the wetting power of the 55 solution to metal and other solid surfaces.

Other objects of this invention will appear from the following description and claims.

Solutions of certain salts of inorganic acids have heretofore been used in cooling systems of automobiles and while some of these salt mixtures have had no decidedly corrosive action upon iron, yet it has been found that they are very corrosive of aluminum and some other metals frequently employed in connection with circulating systems of internal combustion engines. 5 and the like, so that the use of such salt solutions had to be discontinued.

I have found that a very desirable antifreezing liquid can be produced by employing solutions 15 of alkali metal salts of certain organic acids. I have found that the sodium and potassium salts of fatty acids containing not more than nine carbon atoms per molecule, when dissolved in sufficient quantities of water to lower the freezing point of the solution materially below that 20 of water, are substantially no more corrosive of metals than ordinary city water and have very desirable additional properties, namely, that solutions of some of these salts can be produced 25 which can be readily circulated in ordinary circulation systems at temperatures of  $-50^{\circ}$  C. and even lower, that the low temperature solubilities, 30 for example, of potassium acetate, are high enough so that the increases in concentration normally occurring in practice will not cause separation of solid salt at low temperatures even in solutions having very low freezing points, and also that to these solutions can be added effective 35 corrosion inhibitors. These solutions are also compatible with substances for reducing the wetting power of the salt solutions to metal and other surfaces. I have also found that these salts, which in their pure states are often decidedly alkaline in reaction, may have their corrosion 40 action in certain instances very materially reduced by rendering these solutions less alkaline, for example, by the addition of a suitable acid.

Potassium and sodium acetate, the corresponding formates, propionates, butyrates, and corresponding salts of other fatty acids containing not 45 more than nine carbon atoms per molecule are very desirable for use in connection with liquids of this kind. Since solutions of any of these salts in their pure form are often decidedly alkaline in reaction, I may prefer to reduce the alkalinity of these solutions to avoid attack on metals, such for example, as aluminum. In order to prevent possible reactions in the solutions, I prefer to use for this purpose a suitable acid, 50 for example, the acid of the salt in question, 55

- although other acids may be employed, if desired, providing that they do not react with ingredients of my improved antifreeze liquid nor with the metals with which the liquid contacts 5 when in use. In order to buffer these solutions so that they will resist any tendency to change their pH value, a small amount of any of the common buffer mixtures may be added, for example, a small amount of boric acid mixed with 10 its alkali metal salt, or an alkali metal phosphate mixture, may be used. This makes it possible to maintain a solution substantially at a desired pH, even if the water used in diluting the solution is of alkaline or acid reaction.
- 15 The slightly alkaline salt solutions of this kind in any concentration do not attack metals detectably more than ordinary city water does and the salts are also very readily soluble in water, so that if all of the water of the solution is boiled off or evaporated, the residue can be readily dissolved in water, which is very desirable to free 20 a circulating system of the residue, in the event that an antifreezing liquid becomes boiled down or evaporated to dryness.
- 25 In addition to the very desirable characteristics of being readily soluble in water and of being substantially non-corrosive of metals commonly employed in cooling systems, these solutions also have the desirable property of having solidifying 30 points far below that of water. Aqueous solutions of these salts are miscible with alcohol, glycerol and glycols, which is a desirable feature in the event that my improved solution should be added to solutions of these materials. My 35 improved solutions also have the advantage that they can be sold in the form of concentrates and diluted for use by the addition of water thereto, and furthermore, these solutions can be produced at lower cost than glycols and are far more stable 40 than alcohols or glycols with respect to heat or oxidation or reduction.
- Small quantities, for example from  $\frac{1}{4}\%$  to 1% of almost any of the well known corrosion 45 inhibitors may be used in connection with solutions of these salts. Examples of corrosion inhibitors which may be used in connection with my antifreezing liquids are certain organic nitrogen compounds such as urea and amino acridine derivatives. Arsenious oxide, chromates, such as 50 sodium or potassium chromates, and potassium antimony tartrate may also be used.
- I have also found that anti-pyrine constitutes 55 an excellent inhibitor of corrosion, not only for use with my improved antifreeze solutions, but also for use with other solutions. This substance has the formula  $C_{11}H_{12}ON_2$ , and has the peculiarity that in the same a nitrogen atom is bonded to another nitrogen atom. Derivatives of anti-pyrine may also be used as inhibitors of 60 corrosion and the word "anti-pyrine" as herein used is intended to include anti-pyrine and its derivatives. Small quantities of anti-pyrine may be used to effectively prevent corrosion of metals, from  $\frac{1}{4}\%$  to 1% being ordinarily sufficient.
- 65 My improved antifreezing solutions are also compatible with many of the well known materials used to reduce the wetting power of solutions to metals, and preferably not more than about 4% of such material is used in the final solution 70 so that the same will not readily penetrate or seep through small leaks and so that the same will not tend to spread over solid surfaces. By way of example, an animal, mineral or vegetable oil may be used.
- 75 One of the advantages of my improved anti-

freeze solution is that such oils may be readily mixed with the solution without the use of the usual wetting or emulsifying agents. If found desirable in certain cases, wetting or emulsifying agents may be used. Such emulsifying or wetting agent may be soap, an ethanolamine, calcium oleate, magnesium oleate, gum arabic or rosin, or any one of a number of well known materials having a similar action. Preferably mineral oil, such as a light petroleum oil, is used 10 only in conjunction with an approximately equal quantity of an animal or vegetable oil, or all or a part of the light mineral oil can be replaced by an oil of good dielectric properties and high density, such for example as trichlor benzene, 15 chlorinated diphenyl or a phenyl ether. These high density oils can be mixed in such proportions with the animal or vegetable oil as to obtain an oil mixture of the same density as the solution, thus forming a more stable emulsion. The use 20 of an animal or vegetable oil which contains some free fatty acid may be desirable in some cases. In order to obtain the best results, the mixture of the water solution of the salt containing an emulsifying or wetting agent and oil 25 may be passed through a colloid mill to thoroughly homogenize the mixture, so that the oil and water will not separate out on standing, and so that emulsions with air will not be formed as when ordinary mixing its used. When a solution is provided with a material of this nature to reduce the wetting power of the solution to solid surfaces, such solution will not cause trouble with the ignition system of an engine, partly because it collects in drops and does not creep over the 30 surface, and partly because of the nonconducting 35 properties of the oils.

The addition of oils to the salt solution assists in protecting the metals against corrosion. Consequently, if a material of this kind is added 40 to the solution to reduce the wetting power thereof to metal and other solid surfaces, it is frequently unnecessary to use an inhibitor of corrosion.

Potassium acetate is very desirable for use in 45 connection with liquids of this kind, since it very decidedly lowers the freezing or solidifying point of the solution. I have found, for example, that if 3.0 pounds of potassium acetate are made up with water to a total volume of one gallon, the 50 resulting solution will not freeze or solidify at a temperature above  $-24^{\circ} C.$ , and if 5.0 pounds of this salt are made up with water to a total volume of one gallon, the temperature may be lowered to about  $-55^{\circ} C.$  without interfering 55 with the free circulation of the solution. It should be pointed out in this connection that the freezing points of many of these solutions are somewhat indefinite and the temperatures here given represent the highest temperatures at 60 which cloudiness appears in the solution, it being understood that the solutions do not in most cases by any means become entirely solid at these temperatures. Since commercial potassium acetate may have a pH value of about 10, I may prefer 65 to reduce the pH value to about 8 to 9 by adding any organic acid whose potassium salt will not be materially less soluble than potassium acetate. Preferably acetic acid is used for neutralizing potassium acetate. This slightly alkaline salt 70 solution, regardless of its concentration, will not attack metals detectably more than city water does. If the water is boiled off or evaporated from the solution, the residue is in the form of a light fluffy substance and not a compact solid 75

and this substance is, consequently, readily penetrated by and quickly dissolved in water and other liquids. This is a decided advantage over calcium chloride and magnesium chloride which were heretofore used in connection with the formation of antifreezing solutions, which form hard compact masses when the solutions are evaporated to dryness. These compact masses are very hard to redissolve, especially when filling narrow passages. Potassium acetate is sufficiently soluble in water so that it can be marketed in the form of a concentrate containing 10 grams of commercial salt per 10 cc. of solution. This concentrated solution will not crystallize out until temperatures of about  $-15^{\circ}$  C. are reached, and hence the concentrated solutions are practical for shipment and storage. If it is desired to lower the crystal point of the concentrate, this may be done by adding small quantities of alcohol, acetone and other materials. For use in a circulating system, the concentrated solutions when diluted with equal quantities of water form solutions having solidifying points sufficiently low so that they may be circulated readily at temperatures of  $-50^{\circ}$  C.

By way of example, a very excellent antifreezing liquid employing potassium acetate may be formed as described in the following example and adhering to the proportions therein stated:

### Example 1

10 grams of commercial potassium acetate are dissolved in 3 grams of water containing 0.05 gram of anti-pyrine and enough acetic acid to reduce the pH of the solution to about 8 to 9. If desired to buffer this solution, .02 gram of boric acid and .006 gram of potassium hydroxide are added to the solution. To this solution is then added any one of the following materials to reduce wetting power.

- (a) 0.15 cc. to 1 cc. raw linseed oil.
  - (b) 0.3 cc. raw linseed oil plus 0.3 cc. light petroleum oil of low pour point.
  - (c) 0.3 cc. lard oil plus 0.3 cc. light petroleum oil of low pour point.
  - (d) .15 cc. of lard oil, .15 cc. trichlor benzene and .01 gram gum arabic.

The mixture is preferably then passed through a colloid mill or otherwise thoroughly mixed.

50 In this example, if the solution is slightly alkaline, for example, with a pH approximately between 8 and 9, the antipyrine or other corrosion inhibitor may be omitted.

55 This results in the formation of a concentrate which when diluted by adding an equal volume of water will be usable as a circulating medium to temperatures down to  $-46^{\circ}$  C. or lower.

An effective antifreezing liquid may also be made by using potassium formate which acts in a manner very similar to potassium acetate in antifreeze solutions. Potassium formate has the advantage of being somewhat more soluble in water at ordinary temperature than potassium acetate. A very satisfactory antifreeze liquid using potassium formate may be made according to the following example:

*Example II*

6.7 grams of slightly alkaline potassium formate is dissolved in 2.6 grams of water and to the resulting solution 0.03 gram of potassium antimony tartrate are added. The resulting liquid is then homogenized with 3 cc. of the oils specified in connection with Example I to reduce the wetting power of the resulting liquid. This will

make a total volume of about 6.3 ccs. This concentrate can then be made up to a total volume of 10.3 ccs. with water and can be used in a cooling circuit down to a temperature of  $-50^{\circ}$  C. Even at somewhat lower temperatures, the liquid 5 does not completely solidify.

Sodium acetate and sodium formate may be employed for producing antifreezing solutions having very desirable noncorrosive properties and embodying many of the advantages of the corresponding potassium products, except that the solidifying or freezing points of the solutions are somewhat higher and consequently, the corresponding sodium products cannot be used where extremely cold conditions are encountered. Antifreezing liquids employing these sodium salts may be made in accordance with the following examples:

*Example III*

30 grams of slightly alkaline sodium acetate is dissolved in 100 grams of water containing 1 gram of triethanolamine. The resulting solution is then homogenized or thoroughly mixed with 3 grams of lard oil. The resulting solution can be satisfactorily used in a cooling system to temperatures as low as  $-18^{\circ}\text{ C}$ . 20 25

*Example IV*

To a mixture of 25 grams of slightly alkaline sodium formate and 0.7 gram of arsenious oxide is added 75 grams of water. To this solution are added 3 grams of raw linseed oil. The resulting liquid can also be used at temperatures down to  $-18^{\circ}\text{ C}$ . 30

In the case of both Examples III and IV, the liquids formed in accordance with these examples are ready for use in a cooling circuit without diluting with water.

It will be understood that the foregoing examples are merely illustrative and may be varied considerably without departing from this invention. It should also be borne in mind that commercial alkali metal acetates and formates are often not pure and often contain some water, such as water of crystallization, so that the amount of water added may vary accordingly. It will also be obvious that in the event that it is not necessary to employ a solution of reduced wetting power, then the wetting power reducing agent may be omitted, and furthermore, very satisfactory antifreezing preparations can be formed without any corrosion inhibitors. If, for example, the liquid is to be used in contact only with aluminum, the corrosion inhibitors herein described are unnecessary, providing that the salt solution is only slightly alkaline. It will also be obvious that mixtures of the salts herein described may be used to produce antifreeze liquids.

Although the acetates and formates are preferably used because of their relatively low cost, the higher fatty acid salts may be used. In spite of expectations to the contrary, the alkali metal salts of some of the higher fatty acids herein mentioned are even more soluble than the salts of some of the lower acids. For example, potassium butyrate at 31° C. is soluble to the extent of 297 grams in 100 grams of water. Such solutions have the desirable non-corrosive and other properties of the lower fatty acid salts and may be used in similar manner. 65 70

The antifreezing liquids herein described have a number of advantages in addition to those already stated. These salts do not boil away and repeated boiling down or evaporating of solu- 75

tions of the salts and again restoring the water does not change the freezing points of the solutions, nor does it change the property of the liquid of being non-corrosive to metals. The liquids herein described are also very desirable for use as antifreeze solutions in that these solutions either alone or with the oil for reducing the wetting power do not loosen old rust in a cooling system. This is a very desirable feature, since otherwise the loosened rust might clog parts of the system, or leaks may be produced by opening rust clogged holes.

The viscosities at low temperatures of solutions of potassium acetate and formate at the concentrations necessary are much lower than the viscosities at equal temperatures of glycol or glycerol solutions capable of withstanding the same low temperatures. Consequently, these solutions can be circulated more readily at very low temperatures than corresponding glycerol or glycol solutions. Consequently, potassium acetate, potassium formate, and potassium propionate solutions can be used at temperatures materially lower than temperatures at which glycerol or glycol solutions may be used.

An important advantage of my improved anti-freeze liquids is that the maximum boiling point, for example, of potassium acetate solutions is about 165° C. when the solution is boiled down almost to dryness, and this temperature is below the melting point of soft solder. The boiling point of commercial ethylene glycol is over 200° C., which is above the melting point of soft solder. The boiling points of my improved anti-freeze solutions at the concentrations normally used are only slightly higher than the boiling point of water.

Further advantages of my improved antifreeze liquids are that they do not affect the finishes ordinarily employed on automobiles and are particularly inert with reference to lacquer finishes, whereas alcohol and glycols attack such finishes. My improved antifreeze solutions also have no effect upon rubber nor upon synthetic resin products, such as may be used in gaskets or other parts of cooling systems, and furthermore, my improved liquids do not foam when boiling. The salt solutions herein described have the further advantage that they have a higher heat conductivity than glycol or alcohol solutions.

I claim as my invention:

1. The method of cooling metal surfaces which comprises circulating in contact therewith and with cooling surfaces an aqueous solution of high heat conductivity that starts to freeze substantially below 0° C. and can be circulated freely at any temperature above its freezing point; that is stable against oxidation and may be evaporated to dryness without foaming or decomposition or attaining a vapor temperature above 165° C. and the solids of which may then be readily redissolved in water; that will not attack lacquers; that is not substantially more corrosive to iron than ordinary city water and will not change appreciably in this respect upon repeated concentration and redilution; and that is compatible with common corrosion inhibitors and pH buffering agents, and emulsifiable with common animal, vegetable and mineral oils, containing as a major essential ingredient at least one salt of the group consisting of the alkali metal salts of formic, acetic, propionic and butyric acids.

2. In a heat exchange system, an aqueous cooling composition of high heat conductivity that

starts to freeze substantially below 0° C. and can be circulated freely at any temperature above its freezing point; that is stable against oxidation and may be evaporated to dryness without foaming or decomposition or attaining a vapor temperature above 165° C. and the solids of which may then be readily redissolved in water; that will not attack lacquers; that is not substantially more corrosive to iron than ordinary city water and will not change appreciably in this respect with repeated concentration and redilution; and that is compatible with common corrosion inhibitors and pH buffering agents and emulsifiable with common animal, vegetable and mineral oils, containing as a major essential ingredient at least one salt of the group consisting of the alkali metal salts of formic, acetic, propionic, and butyric acids.

3. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming or decomposition or attaining a vapor temperature above 165° C. and the solids of which may then be readily redissolved in water; that will not attack lacquers; that is not substantially more corrosive to common metals than ordinary city water and will not change appreciably in this respect with repeated concentration and redilution; and that is compatible with common corrosion inhibitors and pH buffering agents and emulsifiable with common animal, vegetable and mineral oils, containing as a major essential ingredient a salt of the group consisting of the alkali metal salts of formic, acetic, propionic and butyric acids admixed with a suitable acid in amount sufficient to reduce the alkalinity of the composition in the dilution in which it has the stated freezing characteristics to a pH of substantially 8 to 9.

4. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming or decomposition or attaining a vapor temperature above 165° C. and the solids of which may then be readily redissolved in water; that will not attack lacquers; that is not substantially more corrosive to common metals than ordinary city water and will not change appreciably in this respect with repeated concentration and redilution; and that is compatible with common corrosion inhibitors and pH buffering agents and emulsifiable with common animal, vegetable and mineral oils, containing as a major essential ingredient a salt of the group consisting of the alkali metal salts of formic, acetic, propionic and butyric acids admixed with acid corresponding to the acid radical of said salt in amount sufficient to reduce the alkalinity of the composition in the dilution in which it has the stated freezing characteristics to a pH of substantially 8 to 9.

5. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming or de-

- composition or attaining a vapor temperature above 165° C. and the solids of which may then be readily redissolved in water; that will not attack lacquers; that is not substantially more 5 corrosive to iron than ordinary city water and will not change appreciably in this respect with repeated concentration and redilution; and that is compatible with common corrosion inhibitors and emulsifiable with common animal, vegetable and mineral oils, containing as a major 10 essential ingredient at least one salt of the group consisting of the alkali metal salts of formic, acetic, propionic and butyric acids, stabilized by a buffering agent of the group consisting of boric acid mixed with its alkali metal salt and alkali metal phosphates.
6. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without decomposition or attaining a vapor temperature above 165° C. and 15 the solids of which may then be readily redissolved in water; that will not attack lacquers; that is substantially non-corrosive to iron and will not change appreciably in this respect with repeated concentration and redilution; and that is compatible with common pH buffering agents and emulsifiable with common animal, vegetable, and mineral oils, containing as a major essential 20 ingredient at least one salt of the group consisting of the alkali metal salts of formic, acetic, propionic and butyric acids admixed with a suitable acid in amount sufficient to reduce the alkalinity of the 25 composition in the dilution in which it has the stated freezing characteristics to a pH of substantially 8 to 9, the pH being stabilized with a pH buffering agent.
7. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming, decomposition or attaining a vapor temperature above 165° C. and the solids of which may be readily redissolved in water; that will not attack lacquers 30 or loosen existing rust; that is substantially non-corrosive to iron and will not change appreciably in this respect with repeated concentration and redilution; and that is compatible with common pH buffering agents, and will not creep over 35 metal surfaces, consisting essentially of an emulsion of a solution of at least one salt of the group consisting of the alkali metal salts of formic, acetic, propionic and butyric acids, as a major essential ingredient, with a material of the group 40 consisting of animal, vegetable and mineral oils.
8. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming, decomposition or attaining a vapor temperature above 165° C. and the solids of which may be readily redissolved in water; that will not attack lacquers or loosen existing rust; that is substantially non-corrosive to iron and will not change appreciably in this respect with repeated concentration and redilution; and that is compatible with common pH buffering agents, and will not creep over metal 45 surfaces, consisting essentially of an emulsion of a solution of at least one salt of the group consisting of the alkali metal salts of formic, acetic, propionic and butyric acids, as a major essential ingredient, with a material of the group 50 consisting of animal, vegetable and mineral oils, containing as a major essential ingredient at least one salt of the group consisting of the alkali metal salts of formic, acetic, propionic and butyric acids, stabilized by a buffering agent of the group consisting of boric acid mixed with its alkali metal salt and alkali metal phosphates.
9. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming or decomposition or attaining a vapor temperature above 165° C. and the solids of which may then be readily redissolved in water; that will not attack lacquers; that is substantially non-corrosive to common metals and will not change appreciably in this respect with repeated concentration and redilution; and that is compatible with common corrosion inhibitors and emulsifiable with common animal, vegetable and mineral oils; 55 containing as a major essential ingredient at least one salt of the group consisting of the alkali metal salts of formic, acetic, propionic and butyric acids admixed with a suitable acid in amount sufficient to reduce the alkalinity of the composition in the dilution in which it has the stated freezing characteristics to a pH of substantially 8 to 9, the pH being stabilized with a pH buffering agent.
10. A composition which in suitable aqueous dilution produces a medium for heat transfer, to and from metal surfaces, of high heat conductivity; that starts to freeze below -30° C. and may be circulated freely at any higher temperature; that is stable against oxygen and may be evaporated to dryness without foaming or decomposition or attaining a vapor temperature above 165° C. and the solids of which may then be readily redissolved in water; that will not attack lacquers or loosen existing rust; that is substantially non-corrosive to common metals and will not change appreciably in this respect with repeated concentration and redilution; and that will not readily creep over metal surfaces; 60 consisting essentially of an emulsion of aqueous solution of at least one salt of the group consisting of the alkali metal salts of formic, acetic, propionic and butyric acids, with a minor proportion of an oily material, said emulsion containing a suitable acid in amount sufficient to reduce the alkalinity of the composition in the dilution in which it has the stated freezing characteristics to a pH of substantially 8 to 9, the pH being stabilized with a pH buffering agent.
11. A composition which when dissolved in water to the concentration of substantially 3 pounds of the composition per gallon of solution will produce a medium for heat transfer, to and from metal surfaces, that starts to freeze below -24° C. and may be circulated freely at any higher temperature; may be evaporated to dryness without foaming or decomposition or attaining a vapor temperature above 165° C. and the solids of which may then be readily redissolved in water; that will not attack lacquers; that is not substantially more corrosive to common metals than ordinary city water and will not change appreciably in this respect with repeated concentration and redilution; and that is compatible with common corrosion inhibitors and pH 65 buffering agents.

- buffering agents and emulsifiable with common animal, vegetable and mineral oils, containing as a major essential ingredient potassium acetate admixed with acetic acid in amount sufficient to reduce the alkalinity of the composition in the stated concentration to a pH of substantially 8 to 9.
12. A composition which when dissolved in water to the concentration of substantially 5 pounds of the composition per gallon of solution will produce a medium for heat transfer, to and from metal surfaces; that starts to freeze below  $-55^{\circ}\text{ C}$ . and may be circulated freely at any higher temperature; may be evaporated to dryness without foaming or decomposition or attaining a vapor temperature above  $165^{\circ}\text{ C}$ . and the solids of which may then be readily redissolved in water; that will not attack lacquers; that is not substantially more corrosive to common metals than ordinary city water and will not change appreciably in this respect with repeated concentration and redilution; and that is compatible with common corrosion inhibitors and pH buffering agents and emulsifiable with common animal, vegetable and mineral oils, containing as a major essential ingredient potassium acetate admixed with acetic acid in amount sufficient to reduce the alkalinity of the composition in the stated concentration to a pH of substantially 8 to 9.
13. A liquid composition which will not crystallize out above  $-15^{\circ}\text{ C}$ . and which when diluted with an equal quantity of water will produce a medium for heat transfer, to and from metal surfaces, that starts to freeze below  $-50^{\circ}\text{ C}$ . and may be circulated freely at any higher temperature; that may be evaporated to dryness without foaming or decomposition or attaining a vapor temperature above  $165^{\circ}\text{ C}$ . and the solids of which may then be readily redissolved in water; that will not attack lacquers; that is not substantially more corrosive to iron than ordinary city water and will not change appreciably in this respect with repeated concentration and redilution; and that is compatible with common corrosion inhibitors and pH buffering agents and emulsifiable with common animal, vegetable and mineral oils, consisting essentially of an aqueous solution of potassium acetate, as a major essential ingredient, having a concentration of sub-

stantially 10 grams of the acetate per 10 cc. of solution.

14. A liquid composition which when diluted with an equal volume of water will produce a medium for heat transfer, to and from metal surfaces, that starts to freeze below  $-4^{\circ}\text{ C}$ . and may be circulated freely at any higher temperature; that is stable against oxygen and may be evaporated to dryness without foaming or decomposition or attaining a vapor temperature above  $165^{\circ}\text{ C}$ . and the solids of which may then be readily redissolved in water; that will not attack lacquers or loosen existing rust; that is substantially non-corrosive to common metals and will not change appreciably in this respect with repeated concentration or redilution; and that will not creep over metal surfaces; containing essentially 10 grams of commercial potassium acetate, 3 grams of water, .02 gram of boric acid reacted with .006 gram of potassium hydroxide, .15 to .3 cc. of material of the group consisting of animal, vegetable and mineral oils, a small quantity of an emulsifying agent and acetic acid in amount sufficient to reduce the alkalinity of the composition in the stated final dilution to a pH of substantially 8 to 9.

15. A concentrated liquid composition which when diluted with an equal volume of water will produce a medium for heat transfer, to and from metal surfaces; that starts to freeze below  $-4^{\circ}\text{ C}$ . and may be circulated freely at any higher temperature; that is stable against oxygen and may be evaporated to dryness without foaming or decomposition or attaining a vapor temperature above  $165^{\circ}\text{ C}$ . and the solids of which may then be readily redissolved in water; that will not attack lacquers or loosen existing rust; that is substantially non-corrosive to iron and will not change appreciably in this respect with repeated concentration or redilution; and that will not creep over metal surfaces; containing essentially 10 grams of commercial potassium acetate, 3 grams of water containing 0.05 gram of antipyrine, 1.02 grams of boric acid reacted with .006 gram of potassium hydroxide, .15 to .3 cc. of material of the group consisting of animal, vegetable and mineral oil and a small quantity of an emulsifying agent.